

## UNITED STATES PATENT OFFICE.

ROBERT P. CALVERT, OF MONTCLAIR, NEW JERSEY, ASSIGNOR TO E. I. DU PONT DE NEMOURS & COMPANY, OF WILMINGTON, DELAWARE, A CORPORATION OF DELAWARE.

## NITRATION OF CELLULOSE.

No Drawing. Application filed November 13, 1919, Serial No. 337,847. Renewed February 23, 1922.  
Serial No. 538,773.

To all whom it may concern:

Be it known that I, ROBERT P. CALVERT, a citizen of the United States, and a resident of Montclair, in the county of Essex and 5 State of New Jersey, have invented a certain new and useful Nitration of Cellulose, of which the following is a specification.

This invention relates to a process of nitration cellulose, and pertains particularly 10 to the nitration of tissue paper so treated as to lessen the amount of nitrating acids retainable thereby as a result of capillarity or surface action.

In the nitration of cellulosic materials, 15 there is lost a certain amount of acid through chemical combination with the cellulose and additional amounts in the form of fumes and of acid retained mechanically by the cellulose after wringing. When the cellulose 20 is nitrated in the form of tissue paper this loss of acid through mechanical retention is especially large.

I have found that by compressing the tissue paper, as by passing it through calenders or super-calenders, the amount of acid it 25 will retain mechanically after nitration has been completed is much less than if uncompressed tissue paper had been used.

The compression to which the tissue paper 30 should be subjected by the calenders should be sufficient to substantially reduce its thickness. I preferably compress the paper to approximately half of its former thickness.

The expression "tissue paper" is meant to 35 cover any kind of thin paper into which cellulose is made before nitration. As an example, there may be used tissue paper which is made by pulping rag cuttings with water and then forming the pulp into paper of 40 thickness approximately ".0022" and having a weight of 13 to 15 pounds per ream.

A specific example of the process follows: 45 Tissue paper such as is made from cotton rags is compressed to about half its former thickness by passing it through calenders or super-calenders, is shredded into small pieces, and is then dried to a moisture content of 5% or less. Twenty pounds of the dried paper is then fed into an iron pot containing 1200 lbs. of mixed acid of the approximate composition of 60% sulfuric acid, 50 20% nitric acid and 20% water. After thirty minutes' contact between the acid and

the paper, the entire charge is dumped into a centrifugal which serves to remove most 55 of the acid. The remaining acid is removed by washing.

Analysis of the mixed and spent acids combined chemically or retained mechanically by the nitrocellulose are about as follows, comparison being made with pyroxylon made from compressed and from uncomplicated paper:

*Acid combined chemically and retained mechanically by 65  
1 lb. nitrocellulose (11.1% nitrogen).*

| Kind of paper used. | Nitric acid (basis 100% HNO <sub>3</sub> ). | Sulfuric acid. | 70 |
|---------------------|---------------------------------------------|----------------|----|
| Compressed.....     | 1.0                                         | 1.1            |    |
| Uncompressed.....   | 1.3                                         | 1.2            |    |

It will thus be seen that the saving in concentrated acid is about four-tenths of a 75 pound for each pound of nitrocellulose produced.

I claim:

1. The process of nitrating cellulose which comprises subjecting a thin sheet of cellulose 80 to high compression, shredding the cellulose sheet and treating it with a nitrating acid mixture.

2. The process of nitrating tissue paper which comprises passing it through calenders under a pressure sufficient to materially 85 reduce its thickness, and subjecting the compressed paper to the action of a nitrating acid mixture.

3. The process of nitrating tissue paper 90 which comprises passing it through calenders under a pressure sufficient to materially reduce its thickness, shredding it into small pieces, drying it to a moisture content of not more than 5%, treating it with an excess of 95 a nitrating mixture of sulfuric and nitric acids, centrifugally separating as much strong acid from the nitrated paper as is practicable, and then removing acid remaining in the nitrated paper by washing.

4. In the process of nitrating cellulose, the preliminary step which comprises subjecting a thin sheet of said cellulose to high compression.

5. In the process of nitrating tissue paper, 105 the step which comprises subjecting said

paper to a compression sufficient to materially reduce its thickness.

6. In the process of nitrating tissue paper, the step which comprises passing said paper through calenders under such pressure as to reduce it to about half its former thickness.

7. In the process of nitrating tissue paper,

the steps which comprise passing said paper through calenders under such pressure as to 10 reduce it to about half its former thickness, and then shredding the compressed paper into small pieces.

In testimony whereof I affix my signature.

ROBERT P. CALVERT.